

1

3,404,090

### WATER BASE LUBRICANT

Roy J. Betty, Chicago, Ill., and Robert E. Malec, Birmingham, Mich., assignors to Armour and Company, Chicago, Ill., a corporation of Delaware  
No Drawing. Feb. 14, 1967, Ser. No. 615,924  
4 Claims. (Cl. 252—47.5)

### ABSTRACT OF THE DISCLOSURE

A pyrimidine thione and amine oxide composition for use as a water base lubricant and a process for imparting lubricity to aqueous systems.

### BACKGROUND OF THE INVENTION

This invention pertains to a composition comprising an N-secondary-aliphatic-hexahydropyrimidine-2-thione, and a bis(2-hydroxyethyl) aliphatic amine oxide; and a process utilizing said composition for imparting lubricity to aqueous systems.

In various fields where lubricants are required, it has been found that organic oils are not completely satisfactory. For example, in secondary oil recovery systems, wherein water is pumped into the ground to force oil to the surface, there is a tendency for oil lubricants to plate out upon the pump. Further, when oils are used as cutting fluids, considerable time is often spent in removing the oils from the product. In addition, organic oils may present a fire hazard, they often form emulsions, and they may not be compatible with other additives to the water systems. Also organic oils, such as mineral oil, tend to lose lubricity under certain light and pressure conditions.

Recently, a water base lubricant comprising water and bis(2-hydroxyethyl) aliphatic amine oxides has been disclosed.

### SUMMARY OF THE INVENTION

We have discovered that combining bis(2-hydroxyethyl) aliphatic amine oxides with N-secondary-aliphatic hexahydropyrimidine-2-thiones results in a composition exhibiting synergistic water soluble lubricity. We were surprised to find that this combination imparts water soluble lubricant properties greater than would be expected if the compounds acted independently when used at the same total quantitative amounts. It should be understood that synergistic activity is a relatively rare and unexpected occurrence. Further, our synergistic composition is non-inflammable and is compatible with organic additives such as antifreeze materials, corrosion inhibitors, thickeners, and other desirable additives to the water. In addition, organic oils may be omitted from our process for imparting lubricity to water systems, thereby there is no danger of rancidity, forming of sludge or other degradation products.

Therefore, it is an object of this invention to provide a new composition having utility as a water base lubricant. Another object of this invention is to provide a water base lubricant composition that exhibits synergistic lubricity and is compatible with organic additives such as antifreeze materials, corrosion inhibitors, thickeners, etc. Still another object is to provide a water base lubricant that is light and pressure stable. A further object is to provide a process for imparting lubricity to aqueous systems by means which do not require the addition of organic

2

oils. Other objects and advantages will become more apparent from the ensuing description and examples.

### DETAILED DESCRIPTION OF THE INVENTION

A specific embodiment of our invention may be exemplified by the composition comprising (A) N-(C<sub>7</sub>—C<sub>9</sub> sec-alkyl)hexahydropyrimidine-2-thione and (B) bis(2-hydroxyethyl)cocoamine oxide. While substantial synergistic lubricity is exhibited when the proportions by weight of component (A) to component (B) of this composition range from about 1:5 to about 5:1, particularly desirable results are obtained as the proportions approach 1:1, such as at 3:1, 1:3, 2:1, 1:2 and 1:1. It will be understood that proportions outside this range will exhibit some degree of lubricity.

In another embodiment of our invention, we introduce into water at least 20 parts, per million parts of water by weight, of (A) an N-sec-alkyl-hexahydropyrimidine-2-thione wherein the secondary-alkyl radical contains from 6 to 15 carbon atoms and (B) a bis(2-hydroxyethyl) aliphatic amine oxide wherein the aliphatic radical contains from 6 to 22 carbon atoms, the proportions of (A) to (B) being as illustrated for the composition set forth hereinabove. A preferred concentration of the pyrimidine thione and amine oxide composition is about 50 to 150 parts of the composition per million parts of water, and the upper limits of this concentration do not appear critical. We may use 500 parts of the amine oxide-pyrimidine thione compositions, or more, per million parts of water.

Illustrative amine oxides having utility as one component in our composition have the structure

### FORMULA I



wherein R is an aliphatic hydrocarbon radical containing from 6 to 22 carbon atoms. R may be straight or branched chain, saturated or unsaturated groups such as octyl, nonyl, N-(C<sub>7</sub>—C<sub>9</sub> sec-alkyl), dodecyl, tridecyl, tetradecyl, pentadecyl, N-(C<sub>11</sub>—C<sub>15</sub> sec-alkyl), hexadecyl, octadecyl, octadecenyl, octadecatrienyl, docosyl, eicosyl, and mixtures of radicals such as are derived from naturally occurring glycerides such as coconut oil, tallow, soybean oil and the like. Coconut oil contains a mixture of saturated and unsaturated aliphatic hydrocarbon radicals from C<sub>6</sub> to C<sub>18</sub> and is primarily N-dodecyl. Tallow contains a saturated and unsaturated mixture from C<sub>12</sub> to C<sub>20</sub>, primarily N-hexadecyl, N-octadecyl and octadecenyl. Soybean contains a saturated and unsaturated mixture from C<sub>14</sub> to C<sub>20</sub>, primarily octadecenyl and octadecadienyl.

The preparation of useful bis(2-hydroxyethyl) aliphatic amine oxides may be by the reaction with an excess of hydrogen peroxide as is known in the art.

Exemplary N-sec-alkyl hexahydropyrimidine-2-thiones useful as the second component of our synergistic combination have the structure

### FORMULA II



wherein R is an individual or mixed chain length N-sec-

ondary-alkyl radical having from 6 to 15 carbon atoms. These compounds may be prepared by reacting a thiocarbonyl group containing compound, such as carbon disulfide, thiophosgene, ethylene trithiocarbonate, and the like materials, with a long chain diamine in a mutual solvent, such as methanol, ethanol, isopropanol, butanol, chloroform, ethylene chloride, carbon tetrachloride, ether and the like materials at temperatures of 0° to 80° C. Some useful diamines for this preparation have the following structure:

FORMULA III



wherein R is a secondary alkyl radical having from 6 to 15 carbon atoms. Initially, the dithiocarbamic acid inner salt is formed which, upon further heating at 90° to 200° C. gives off hydrogen sulfide with formation of the cyclic hexahydropyrimidine-2-thione.

When the composition has been prepared as above described, other additives may be included in the water system. For example, low molecular weight glycols or alcohols, such as ethylene glycol, propylene glycol, etc., or methanol, ethanol, etc., may be added as antifreeze materials. Carboxymethyl cellulose, alginates, etc. may be added as thickeners. Similarly, water corrosion inhibitors may be added. The foregoing additives are compatible with the water base lubricant. If desired, they may be omitted.

Comparative evaluations of the amine oxides and pyrimidine thiones as described herein show that these compounds exhibit greater lubricity in combination than would be expected if the compounds acted independently. A specific comparison is set out in the accompanying examples, which are illustrative of our composition and process.

#### Example I

Equimolar amounts of a mixture of long chain C<sub>7</sub> to C<sub>9</sub> secondary-alkyl diamines and carbon disulfide are admixed with cooling and stirring while both are dissolved in ethanol. The ethanol solution of each comprises a 50% by weight solution. A temperature of 30° C. is utilized as the reaction temperature. A mixture of N-(C<sub>7</sub>-C<sub>9</sub> sec-alkyl)-1,3-propanediamine-N'-dithiocarbamic acids is formed. The acids are then removed from the alcoholic media by evaporation and heated at a temperature of 115° C. to cause evolution of H<sub>2</sub>S. This causes cyclization to N-(C<sub>7</sub>-C<sub>9</sub> sec-alkyl)hexahydropyrimidine-2-thione.

#### Example II

A convenient and meaningful method of measuring water soluble lubricity is by means of a Baroid extreme pressure mud tester, which is similar to a Timken wear tester. A standard evaluation procedure is followed wherein the test cup and the test block are weighed to the nearest mg.; then the test cup is mounted on the beveled ring located on the bottom of the belt driven shaft and the test block is mounted at the bottom of the shaft connected to the torque arm. The sample container is filled with approximately 200 ml. of a brine solution or tap water with the desired amount of the chemical to be evaluated. After the sample cup is positioned so that the test cup and test block are covered with fluid, the motor is started and the machine allowed to run 5 minutes with no load applied. The "load test" evaluation is then started at 20 lb. load and taken up to 140 lb. load in 20 lb. increments at 5 minute intervals. The "wear test" evaluation is the same evaluation initially, with a continuation of running the machine at 140 lb. load for 30 minutes. At the end of the evaluation test periods, the test cup and block are removed, rinsed, and reweighed. The weight loss (amount of wear) indicates the efficiency of the lubricant. If galling or seizing occurs during the evaluation, the machine is stopped. The brine solution used in

some of the evaluations following herein consisted of 80% water, 10.5% sodium chloride, 9.4% calcium chloride, 0.06% magnesium chloride, 0.02% ferric chloride, and 0.02% sodium sulfate.

Illustrative results comparing a known water soluble lubricant and certain of the components of this invention, individually and combined, are set forth in Table I. The chemicals designated in the table are defined as follows:

- 10 Aromox C/12 is bis(2-hydroxyethyl)cocoamine oxide  
 Aromox T/12 is bis(2-hydroxyethyl)tallowamine oxide  
 NL-7 PTU is N-(C<sub>7</sub>-C<sub>9</sub> sec-alkyl)hexahydropyrimidine-2-thione  
 NL-11 PTU is N-(C<sub>11</sub>-C<sub>15</sub> sec-alkyl)hexahydropyrimidine-2-thione.

TABLE I

|                                | Chemical | Concentration, p.p.m. | Wear in mg. weight loss |
|--------------------------------|----------|-----------------------|-------------------------|
| Load test in brine:            |          |                       |                         |
| 20 Standard <sup>1</sup> ----- | 300      | 41.3                  |                         |
| Aromox C/12-----               | 200      | 10.8                  |                         |
| NL-7 PTU-----                  | 100      | 55.5                  |                         |
| NL-11 PTU-----                 | 100      | 25.7                  |                         |
| Aromox C/12 and NL-7 PTU-----  | 50       | 13.9                  |                         |
| Aromox C/12 and NL-11 PTU----- | 100      | 19.8                  |                         |
| Load test in tapwater:         |          |                       |                         |
| 25 Aromox C/12-----            | 200      | 55.5                  |                         |
| NL-7 PTU-----                  | 100      | 30.0                  |                         |
| Aromox C/12 and NL-7 PTU-----  | 100      | 10.2                  |                         |
| 30 Wear test in brine:         |          |                       |                         |
| Aromox C/12 and NL-7 PTU-----  | 100      | 2.1                   |                         |
| NL-7 PTU-----                  | 50       |                       |                         |

<sup>1</sup> A water base lubricating product primarily containing a methyl ester of alpha sulfo stearic acid.

#### Example III

Illustrative proportions and concentrations showing the enhanced water base lubricity of the composition are set forth in the following additional "load test" results obtained by the procedures of Example II:

TABLE II

|                                          | Chemical | Concentration, p.p.m. | Wear in mg. weight loss |
|------------------------------------------|----------|-----------------------|-------------------------|
| 45 Load test in tap water:               |          |                       |                         |
| 67% Aromox C/12 and 33% NL-7 PTU-----    | 100      | 3.5                   |                         |
| 33% Aromox C/12 and 67% NL-7 PTU-----    | 100      | 2.8                   |                         |
| Load test in brine:                      |          |                       |                         |
| 50 50% Aromox C/12 and 50% NL-7 PTU----- | 300      | 3.1                   |                         |
| Do-----                                  | 250      | 2.6                   |                         |
| Do-----                                  | 200      | 1.5                   |                         |
| Do-----                                  | 150      | 1.0                   |                         |
| Do-----                                  | 75       | 6.9                   |                         |
| Do-----                                  | 50       | 10.8                  |                         |

While in the foregoing specification, we have described specific compositions and procedures in considerable detail for the purpose of illustrating our invention, those skilled in the art will appreciate that variations can be made without departing from the spirit and scope of our invention; and therefore, it is not intended to be limited except as indicated in the appended claims.

We claim:

- 65 1. A composition comprising an N-secondary-aliphatic hexahydropyrimidine-2-thione wherein the secondary-aliphatic radical contains from 6 to 15 carbon atoms and a bis(2-hydroxyethyl) aliphatic amine oxide wherein the aliphatic radical contains from 6 to 22 carbon atoms, and in which the proportions by weight of the pyrimidine thione to the amine oxide range from about 1:5 to about 5:1, said composition displaying synergistic lubricity when used with water in a concentration of at least 20 p.p.m.
- 70 2. The composition of claim 1 in which said pyrimidine thione is N-(C<sub>7</sub>-C<sub>9</sub> sec-alkyl)-hexahydropyrimidine-2-

thione and said amine oxide is bis(2-hydroxyethyl)coco-amine oxide and said proportion is about 2:1.

3. The composition of claim 1 in which said composition displays synergistic lubricity when used with brine in a concentration of at least 20 p.p.m.

4. The composition of claim 3 in which said pyrimidine thione is N-(C<sub>7</sub>-C<sub>9</sub> sec-alkyl)hexahydropyrimidine-2-thione and said amine oxide is bis(2-hydroxyethyl)coco-amine oxide and said proportion is about 1:2.

## References Cited

## UNITED STATES PATENTS

3,108,071 10/1963 Harker ----- 252—47 X  
3,346,495 10/1967 Malec et al. ----- 252—49.3

PATRICK P. GARVIN, *Primary Examiner.*

W. H. CANNON, *Assistant Examiner.*